

# United States Patent [19]

Raby et al.

[11] 3,910,836

[45] Oct. 7, 1975

[54] PYROCHLORE FLOTATION

[75] Inventors: Raymond Raby; Clement J. Desrochers, both of Ste. Foy, Canada

[73] Assignee: Soquem, Montreal, Canada

[22] Filed: July 29, 1974

[21] Appl. No.: 492,704

|           |         |               |           |
|-----------|---------|---------------|-----------|
| 2,861,687 | 11/1958 | Lord .....    | 209/166 X |
| 2,875,896 | 3/1959  | Last .....    | 209/166   |
| 2,951,585 | 9/1960  | Burks .....   | 209/167   |
| 2,959,281 | 11/1960 | Faucher ..... | 209/166 X |
| 3,014,585 | 12/1961 | Noblitt ..... | 209/166 X |

OTHER PUBLICATIONS

Chem. Abst., Vol. 69, 1968, 98604x.

Chem. Abst., Vol. 69, 1968, 108831k.

Primary Examiner—Robert Halper

[57] ABSTRACT

An ore containing small amounts of columbium-bearing minerals is beneficiated by froth flotation, an aqueous pulp of the ground ore being floated in the presence of a cationic collector of the amine type, a surface active agent and a modifying agent providing a source of free oxalate ions from the group consisting of oxalic acid and oxalate salts. A concentrate rich in the columbium-bearing minerals is floated off and collected, with a columbium-lean tailing remaining.

8 Claims, 2 Drawing Figures

Related U.S. Application Data

[63] Continuation-in-part of Ser. No. 311,282, Dec. 1, 1972, abandoned.

[30] Foreign Application Priority Data

Jan. 29, 1972 United Kingdom..... 4307/72

[52] U.S. Cl..... 209/166; 209/12

[51] Int. Cl.<sup>2</sup>..... B03D 1/02

[58] Field of Search ..... 209/166, 167, 2, 12, 3

[56] References Cited

UNITED STATES PATENTS

1,912,434 6/1933 Crago ..... 209/166







## PYROCHLORE FLOTATION

This is a continuation-in-part of application Ser. No. 311,282, now abandoned filed Dec. 1, 1972.

## BACKGROUND OF THE INVENTION

This invention relates to the beneficiation by froth flotation of columbium-bearing minerals from ore containing such minerals. It is particularly applicable to those columbium (niobium) ores containing various proportions of carbonates, such as dolomite, calcite, etc.; silicates such as mica, pyroxene etc., and metallic oxides such as ilmenite, hematite, magnetite etc., and other minerals such as apatite, zircon, sulfides, etc.

The invention is most useful in the treatment of ores containing pyrochlore, such as the pyrochlore-bearing ores found in the province of Quebec, Canada, which contain large quantities of gangue materials, including large quantities of carbonates.

There are few processes available for effectively and economically obtaining concentrates of columbium minerals from columbium-bearing ores which are rich enough in columbium content to be commercially useful. In U.S. Pat. No. 2,875,896 columbium minerals are concentrated by froth flotation using a reagent from the hydroxy quinoline group of chemical compounds as a selective collector for columbium minerals. U.S. Pat. No. 2,951,585 discloses a separation of pyrochlore from calcite, apatite and silica by froth flotation in the presence of an aliphatic monoamine or diamine and an improvement in this process is advanced in U.S. Pat. No. 3,014,585 by use of a modifying agent consisting of a water-soluble bicarbonate in the flotation solution. Unfortunately, none of these processes result in a high grade  $\text{Cb}_2\text{O}_5$  concentrate.

In U.S. Pat. No. 2,959,281 a process is disclosed whereby columbium-bearing ores are beneficiated by froth flotation using a cationic promoter of the amine type and a selective activator containing a source of free fluoride and fluosilicate ions.

Russian researches have made unsuccessful efforts to produce suitable pyrochlore concentrates and have used what is referred to as an "1M-50" complexing reagent in association with oxalic acid and sodium silicate. The "1M-50" reagent is obtained by synthesizing higher alkylhydroxamic acids. The Russian mining industry has, however, been forced to resort to chemical processing to produce a columbium product which can be sold on the world market.

It has now been found that columbium-bearing minerals, and particularly those of the pyrochlore type, can be floated from alkaline ores, with a good separation from the gangue constituents utilizing a novel reagent combination comprising a cationic collector of the amine or diamine type emulsified with a surface active agent and a modifying agent, providing a source of free oxalate ions, from the group consisting of oxalic acid and oxalate salts, with or without pH modifier, including any inorganic acid, in an acid circuit.

## SUMMARY

In the process of the invention a low grade ore containing small amounts of columbium-bearing minerals, and in particular pyrochlore, associated with large amounts of gangue, including large quantities of carbonates, is first ground to a particle size suitable for separation of the columbium-bearing minerals by froth flotation and an aqueous pulp of the finely ground ore

is then subjected to froth flotation in the presence of a cationic collector of the amine type, and particularly of the diamine acetate type, advantageously having a carbon chain length of 10 to 22 carbon atoms, a dispersing agent and a modifying agent providing a source of free oxalate ions from the group consisting of oxalic acid and oxalate salts to obtain a concentrate rich in the columbium-bearing minerals and a columbium-lean flotation tailing. Inorganic acids such as hydrochloric, sulfuric and phosphoric are useful in maintaining an acid circuit and gangue depressants such as caustic starch, sodium silicate and lactic acid may be used in the circuit. Furthermore, the addition of  $\text{CaCl}_2$  can be beneficial to the circuit.

The principal object of the present invention is to provide an improved process for the flotation of columbium-bearing minerals from alkaline ores (carbonates) by which a high grade  $\text{Cb}_2\text{O}_5$  concentrate can be obtained.

Other objects and advantages of the invention will be apparent from the description following taken in conjunction with the accompanying drawing in which:

## BRIEF DESCRIPTION OF THE DRAWING

FIG. 1 is a flowsheet of a process embodying the invention; and

FIG. 2 is another flowsheet illustrating a further embodiment of the invention.

## DESCRIPTION OF THE PREFERRED EMBODIMENTS

Referring to FIG. 1 of the drawings and, for illustrative purposes referring to flotation of a pyrochlore concentrate, the ore is crushed and ground to a fineness of -65 mesh and a pulp of the ground ore is deslimed and then conditioned with a cationic collector of the diamine acetate type, and a dispersing agent acting in combination with the collector together with oxalic acid or an oxalate salt. The conditioned pulp is submitted to flotation to obtain a rougher pyrochloric concentrate which is cleaned using the same reagents in a number of cleaning stages. Middlings from such cleaning are re-treated and returned to the rougher flotation step.

The cleaned pyrochlore concentrate is submitted to a sulfide flotation, where necessary, after conditioning with caustic starch and/or sodium silicate along with a suitable xanthate collector, such as potassium amyl xanthate, to obtain a rougher pyrite concentrate which is cleaned, with the cleaner middlings being returned to the pyrochlore concentrate. A second desliming of the pyrochlore concentrate may advantageously be carried out and it is then submitted to further cleaning stages while using the cationic collector, as before, oxalic acid and a gangue depressant. Middlings are returned to the pyrochlore rougher flotation and a high grade  $\text{Cb}_2\text{O}_5$  flotation concentrate is obtained containing as high as 65%  $\text{Cb}_2\text{O}_5$ . It is possible also to carry out reverse flotation of the pyrite after the last  $\text{Cb}_2\text{O}_5$  cleaning stage.

The process of the invention is embodied also in the procedure illustrated by the flowsheet of FIG. 2 in which carbonates and silicates are pre-floated followed by the flotation of pyrochlore using oxalic acid. By this procedure the ore is ground to -65 mesh and a pulp of the ground ore in water is deslimed and conditioned with suitable reagents for a carbonate flotation and then subjected to flotation of a rougher carbonate con-

centrate. This carbonate concentrate is cleaned using similar reagents and the cleaner tails are combined with the rougher tails for subsequent pyrochlore flotation.

The combined tails are deslimed and conditioned with a suitable cationic collector of the diamine acetate type, and a dispensing agent together with oxalic acid. An inorganic acid may be added for pH control, the flotation process being carried out in an acid medium, i.e. at a pH of below 7. A  $\text{Cb}_2\text{O}_5$  rougher concentrate is floated and this concentrate may, if necessary, be subjected to a sulfide flotation after conditioning with a suitable gangue depressant and a suitable xanthate collector. The pyrite rougher concentrate is advantageously cleaned with the middlings being combined with the pyrite rougher tails (pyrochlore concentrate). The pyrochlore concentrate is submitted to a number of cleaning stages using reagents as in the  $\text{Cb}_2\text{O}_5$  rougher flotation and middlings from the cleaning stages are returned to the  $\text{Cb}_2\text{O}_5$  rougher flotation. A high grade  $\text{Cb}_2\text{O}_5$  concentrate is obtained.

It is to be noted that columbium-bearing ores treated according to the process of the invention contain large quantities of silicates or gangue, such as mica, pyroxene, nepheline, melilite and plagioclase, and, in particular, gangue such as the carbonates dolomite, calcite, ankerite and siderite. Minerals such as apatite, fluoride, zircon, sulfides and barite and heavy minerals such as hematite, magnetite and ilmenite may be present. These silicates or gangue, heavy minerals and carbonates are depressed in the flotation by the combined effects of the oxalic acid and a suitable gangue depressant such as caustic starch, sodium silicate, phosphoric acid and lactic acid. In the process it is not necessary to use separate magnetic or gravity separation to eliminate magnetite, ilmenite, rutile, hematite or mica. Mica can be an abundant gangue material associated with pyrochloric and mica is advantageously depressed during the froth flotation using caustic starch, lactic acid or phosphoric acid. The heavy minerals such as ilmenite, hematite and magnetite are depressed by the same depressants as for mica. Carbonates in the ore, such as for example, dolomite, ankerite, calcite and siderite are advantageously depressed in the flotation by the combined effects of the oxalic acid and a suitable gangue depressant, such as caustic starch or sodium silicate. Part or most of the carbonates may, however, as illustrated in the flowsheet of FIG. 2, be pre-floated before flotation of the columbium-bearing minerals.

Although the embodiments of FIGS. 1 and 2 of the drawings have been described with reference to obtaining a pyrite concentrate when floating sulfides from the pyrochlore concentrate, sulfides other than pyrite may be removed by this flotation operation.

As afore-mentioned, the flotation of the columbium-bearing mineral is carried out in an acid circuit, i.e. at a pH of below 7, and acids such as hydrofluoric, sulfuric, hydrochloric and phosphoric may be used as pH modifiers. Hydrofluoric acid may be mixed with the oxalic acid or oxalate salt modifying agent in the flotation operation. An admixture of up to in the order of equal amounts of hydrofluoric acid with oxalic acid appears to be useful. Furthermore, the addition of calcium chloride to the circuit has been found to have some beneficial effects for the pyrochlore flotation.

It is to be noted that it is the novel combination of the cationic collector of the diamine acetate type together with the oxalic acid or oxalate salt modifying agent

which provides the very selective flotation action towards the pyrochlore mineral. Preferably, the diamine acetate collector should be one having a carbon chain length of 10 to 22 carbons or mixtures thereof in order to provide the most effective flotation of the pyrochlore mineral.

The following examples are illustrative of the process of the present invention.

#### EXAMPLE I

##### Direct Pyrochlore Flotation with Oxalic Acid

A sample of pyrochlore-containing ore from the St-Honore district (Chicoutimi) Province of Quebec, Canada, which is associated with dolomite, calcite, apatite, mica, pyroxene, heavy minerals, such as ilmenite, magnetite, hematite and sulfides and normally contains 0.90 to 1.05%  $\text{Cb}_2\text{O}_5$ , was prepared by crushing and grinding to -65 mesh fineness and was treated in accordance with the flowsheet shown in FIG. 1.

A pulp of the ground ore containing about 35% solids in water was deslimed and conditioned for one minute with 0.90 lbs./ton of a properly prepared mixture of 3 parts and 1 part respectively of Duomac-T (trade mark) and Ethofat 242/25 (trade mark) cationic collectors (both produced by Armour Industrial Chemical Co.) and 1.50 lbs./ton of oxalic acid. The Ethofat 242/25 and Ethofat 242/45, referred to hereinafter, are dispersing agents consisting of ethoxylated fatty acids, as defined by Armour Industrial Chemical Co., and they act in combination with the Duomac-T collector to provide the necessary selectivity for pyrochlore.

The conditioned pulp was then submitted to the flotation of a rougher pyrochlore concentrate which was cleaned five times, while adding the following quantities of reagent at the various cleaning stages:

|                         |                       |
|-------------------------|-----------------------|
| Duomac-T Ethofat 242/25 | 0.05 to 0.35 lbs./ton |
| Oxalic Acid             | 0.25 to 0.50 lbs./ton |

40

The concentrate obtained was then submitted to a sulfide flotation after conditioning for five minutes with 0.10 lbs. per ton of caustic starch and 0.15 lbs./ton of sodium silicate along with 0.02 lbs./ton of potassium amyl xanthate. The rougher pyrite concentrate was cleaned three times with the cleaner tailings being returned to the pyrochlore concentrate.

A second desliming was carried out prior to the fifth cleaning stage.

The pyrochlore concentrate was then submitted to four successive cleaning stages while adding the following quantities of reagents at the various cleaning stages.

|                         |                       |
|-------------------------|-----------------------|
| Duomac-T Ethofat 242/45 | 0.0 to 0.05 lbs./ton  |
| Oxalic Acid             | 0.25 to 0.50 lbs./ton |
| Caustic Starch          | 0.00 to 0.05 lbs./ton |
| Sodium Silicate         | 0.00 to 0.10 lbs./ton |

60

The results of this procedure are shown in Table I.

Table No. I

| Products | % Weight | % $\text{Cb}_2\text{O}_5$ | % Recovery |
|----------|----------|---------------------------|------------|
| Slimes   | 12.35    | 0.58                      | 7.9        |
| Rejects  | 38.40    | 0.03                      | 1.2        |

Table No. I-Continued

| Products                            | % Weight | % $\text{Cb}_2\text{O}_5$ | % Recovery |
|-------------------------------------|----------|---------------------------|------------|
| Sulfides                            | 0.60     | 0.60                      | 0.4        |
| Middlings                           | 52.60    | 0.27                      | 15.5       |
| $\text{Cb}_2\text{O}_5$ concentrate | 1.25     | 54.5                      | 75.0       |
| Calculated head                     | 100.00   | 0.91                      | 100.0      |

## EXAMPLE II

A sample similar to that used in Example I, was treated according to the same procedure except oxalic acid addition was reduced and hydrochloric acid was added. The following quantities of reagents were used.

Conditioning for  $\text{Cb}_2\text{O}_5$  Flotation:

|                             |                       |
|-----------------------------|-----------------------|
| Duomac-T Ethofat 242/25     | 0.8 lbs./ton          |
| Oxalic Acid                 | 0.5 lbs./ton          |
| Hydrochloric Acid           | 0.5 lbs./ton          |
| First Five Cleaning Stages: |                       |
| Duomac-T Ethofat 242/45     | 0.03 to 0.15 lbs./ton |
| Oxalic Acid                 | 0.15 to 0.5 lbs./ton  |
| Hydrochloric Acid           | 0.15 to 0.5 lbs./ton  |

## Conditioning for Sulfide Flotation:

|                            |                       |
|----------------------------|-----------------------|
| Causticized Starch         | 0.05 lbs./ton         |
| Sodium Silicate            | 0.10 lbs./ton         |
| Potassium Amyl Xanthate    | 0.02 lbs./ton         |
| Last Four Cleaning Stages: |                       |
| Duomac-T Ethofat 242/45    | 0.0 to 0.05 lbs./ton  |
| Oxalic Acid                | 0.15 to 0.25 lbs./ton |
| Hydrochloric Acid          | 0.15 to 0.25 lbs./ton |
| Causticized Starch         | 0.0 to 0.05 lbs./ton  |
| Sodium Silicate            | 0.0 to 0.10 lbs./ton  |

The final concentrate obtained was leached with an excess quantity of 37% concentrated hydrochloric acid to obtain the final product.

The results of the procedure used in Example II are shown in Table II

Table No. II

| Products                              | % Weight | % $\text{Cb}_2\text{O}_5$ | % Distribution |
|---------------------------------------|----------|---------------------------|----------------|
| Slimes                                | 11.2     | 0.54                      | 6.7            |
| Rejects                               | 48.9     | 0.05                      | 2.6            |
| Sulfides                              | 0.6      | 0.56                      | 0.4            |
| Middlings                             | 37.6     | 0.37                      | 15.5           |
| Flot. $\text{Cb}_2\text{O}_5$ Conc.   | 1.68     | 40.2                      | 74.8           |
| Calculated Head                       |          | 0.90                      | 100.0          |
| Leached $\text{Cb}_2\text{O}_5$ Conc. | 1.15     | 58.8                      | 74.8           |

## EXAMPLE III

A sample similar to that used in Example I was treated according to the same procedure except oxalic acid addition was reduced and phosphoric acid was added.

Conditioning for  $\text{Cb}_2\text{O}_5$  Flotation:

|                             |               |
|-----------------------------|---------------|
| Duomac-T Ethofat 242/25     | 0.7 lbs./ton  |
| Oxalic Acid                 | 0.5 lbs./ton  |
| Phosphoric Acid             | 0.5 lbs./ton  |
| Reagent 825 (Cyanamid)      | 0.25 lbs./ton |
| First Five Cleaning Stages: |               |

10 The final concentrate obtained was leached with an excess quantity of 37% concentrated hydrochloric acid to obtain the final product.

15 The results of the procedure used in Example III are shown in Table III.

Table No. III

| Products                              | % Weight | % $\text{Cb}_2\text{O}_5$ | % Distribution |
|---------------------------------------|----------|---------------------------|----------------|
| Slimes                                | 11.5     | 0.53                      | 7.1            |
| Rejects                               | 52.0     | 0.09                      | 5.0            |
| Sulfides                              | 0.5      | 0.49                      | 0.3            |
| Middlings                             | 34.0     | 0.41                      | 15.7           |
| Flot. $\text{Cb}_2\text{O}_5$ Conc.   | 2.04     | 31.6                      | 71.9           |
| Calculated Head                       | 100.0    | 0.90                      | 100.0          |
| Leached $\text{Cb}_2\text{O}_5$ Conc. | 1.20     | 53.8                      | 71.9           |

35

## EXAMPLE IV

40 A sample of ore similar to the one described in Example I was prepared by crushing and grinding to a -65 mesh fineness and was treated by the procedure illustrated in the flowsheet in FIG. 2 by which the carbonates and silicates are pre-floated followed by flotation of the pyrochlore. The pulp formed containing about 35% solids in water was conditioned for 15 minutes with 1.25 lbs./ton of causticized starch, 1.00 lbs./ton of sodium silicate 1.30 lbs./ton of a fatty acid - Lannagol (trade mark) emulsion and 0.04 lbs./ton of M.I.B.C. (Methyl-Isobutyl-Carbinol). The conditioned pulp was then submitted to the flotation of a rougher carbonate concentrate, which was cleaned four times, while returning the cleaner tails with the rougher tails for subsequent pyrochlore flotation.

45 The following reagents were added at the various carbonate flotation cleaning stages.

55

|                                |                       |
|--------------------------------|-----------------------|
| Caustized Starch               | 0.05 to 1.00 lbs./ton |
| Sodium Silicate                | 0.05 to 1.00 lbs./ton |
| Fatty Acid + Lannagol Emulsion | 0.00 to 0.40 lbs./ton |

60 The carbonate flotation rougher and cleaner tails were then deslimed and submitted to a rougher pyrochlore flotation after a conditioning period of one minute with 0.30 lbs./ton of Duomac-T Ethofat Emulsion and 2.20 lbs./ton of oxalic acid. The tailings were rejected and the rougher concentrate was then submitted

-Continued

to sulfide flotation after conditioning for five minutes with 0.10 lbs./ton of causticized starch, 0.15 lbs./ton of sodium silicate and 0.02 lbs./ton of potassium amyl xanthate.

The pyrite rougher tails (pyrochlore concentrate) was then submitted to four cleaning stages while adding the following reagent at the various cleaning stages:

|                    |                       |
|--------------------|-----------------------|
| Duomac-T Ethofat   | 0.00 to 0.05 lbs./ton |
| Oxalic Acid        | 0.25 to 0.74 lbs./ton |
| Causticized Starch | 0.00 to 0.05 lbs./ton |
| Sodium Silicate    | 0.00 to 0.10 lbs./ton |

The results obtained by the procedure of Example IV are shown in Table IV.

Table No. IV

| Products                            | % Weight | % $\text{Cb}_2\text{O}_5$ | % Distribution |
|-------------------------------------|----------|---------------------------|----------------|
| Carbonates Conc.                    | 54.6     | 0.10                      | 5.4            |
| Slimes                              | 3.3      | 1.50                      | 5.0            |
| Rejects                             | 23.9     | 0.09                      | 2.0            |
| Pyrite Conc.                        | 0.8      | 0.17                      | 0.1            |
| Middlings                           | 16.1     | 0.75                      | 11.6           |
| Flot. $\text{Cb}_2\text{O}_5$ Conc. | 1.3      | 58.50                     | 75.9           |
| Calculated Head                     | 100.0    | 1.03                      | 100.0          |

## EXAMPLE V

A composite sample similar to that used in Example I was treated according to the same procedure as used in that example except that a mixture of hydrofluoric and oxalic acids in a ratio of 1 part HF to 3 oxalic was added and the sulfides were floated off after the seventh  $\text{Cb}_2\text{O}_5$  cleaning stage.

Conditioning for  $\text{Cb}_2\text{O}_5$  Flotation:

|                                     |                       |
|-------------------------------------|-----------------------|
| Duomac-T Ethofat 242/25             | 0.85 lbs./ton         |
| Acid Mixture                        | 0.05 lbs./ton         |
| First Seven Cleaning Stages:        |                       |
| Duomac-T Ethofat 242/25             | 0.02 to 0.35 lbs./ton |
| Acid Mixture                        | 0.25 to 0.50 lbs./ton |
| Causticized                         | 0.00 to 0.05 lbs./ton |
| Sodium Silicate                     | 0.00 to 0.10 lbs./ton |
| Conditioning for Sulfide Flotation: |                       |
| Causticized Starch                  | 0.05 lbs./ton         |
| Sodium Silicate                     | 0.10 lbs./ton         |
| Potassium Amyl Xanthate             | 0.02 lbs./ton         |
| Sodium Hydroxide                    | to alkaline pH        |
| Last Cleaning Stage:                |                       |
| Duomac-T Ethofat 242/25             | 0.01 lbs./ton         |
| Acid mixture                        | 0.50 lbs./ton         |
| Causticized Starch                  | 0.05 lbs./ton         |

The results obtained by this procedure are shown in Table V.

Table No. V

| Products                            | % Weight | % $\text{Cb}_2\text{O}_5$ | % Distribution |
|-------------------------------------|----------|---------------------------|----------------|
| Slimes                              | 7.7      | 0.44                      | 3.8            |
| Rejects                             | 88.1     | 0.08                      | 8.8            |
| Sulfides                            | 0.6      | 0.43                      | 0.3            |
| Middlings                           | 2.0      | 1.62                      | 3.6            |
| Flot. $\text{Cb}_2\text{O}_5$ Conc. | 1.56     | 47.7                      | 83.5           |
| Calculated Head                     | 100.0    | 0.89                      | 100.0          |

## EXAMPLE VI

Example V was repeated except that a mixture of hydrofluoric and oxalic acids in a ratio of 1 part HF to 1 part oxalic acid was used. Otherwise, the same procedure and the same reagents were used as in Example V. The results obtained are shown in Table VI.

Table No. VI

| Products                            | % Weight | % $\text{Cb}_2\text{O}_5$ | % Distribution |
|-------------------------------------|----------|---------------------------|----------------|
| Slimes                              | 6.9      | 0.40                      | 3.0            |
| Rejects                             | 83.3     | 0.07                      | 6.8            |
| Sulfides                            | 0.6      | 0.16                      | 0.1            |
| Middlings                           | 7.7      | 0.59                      | 5.3            |
| Flot. $\text{Cb}_2\text{O}_5$ Conc. | 1.54     | 50.1                      | 84.8           |
| Calculated Head                     | 100.0    | 0.91                      | 100.0          |

It has been found that the use of oxalic acid as a modifying agent in the promotion of the flotation of columbium-bearing minerals, such as pyrochlore, has an advantage over using hydrofluoric acid as a modifying agent in substantially reducing the amount of silica in the pyrochlore flotation concentrate. A series of tests were conducted illustrating this advantage in which the same procedure and the same reagent materials were used, the ore being treated being the same in each test, except that hydrofluoric acid was used as a modifying agent in five of the tests and oxalic acid was used as a modifying agent in nineteen of the tests. In Table VII the present  $\text{Cb}_2\text{O}_5$  and the percent  $\text{SiO}_2$  in the flotation concentrates obtained in each of the tests is given. The results of Table VII show that a concentrate with substantially the same  $\text{Cb}_2\text{O}_5$  content has, on the average, a much lower silica content when using oxalic acid than when using hydrofluoric acid.

Table No. VII

| Hydrofluoric Acid<br>% $\text{Cb}_2\text{O}_5$ | Oxalic Acid<br>% $\text{Cb}_2\text{O}_5$ |
|------------------------------------------------|------------------------------------------|
| % $\text{SiO}_2$                               | % $\text{SiO}_2$                         |
| 47.6                                           | 45.4                                     |
| 43.5                                           | 49.6                                     |
| 47.0                                           | 46.0                                     |
| 46.6                                           | 37.1                                     |
| 38.1                                           | 41.2                                     |
| 44.56                                          | 48.1                                     |
| 6.00                                           | Average                                  |
|                                                |                                          |
| 35.2                                           | 35.38                                    |
| 35.8                                           | 35.38                                    |
| 44.4                                           | 34.47                                    |
| 40.1                                           | 43.44                                    |
| 34.8                                           | 1.18                                     |
| 38.2                                           | 0.48                                     |
| 43.1                                           | 2.14                                     |
| 50.8                                           | 0.98                                     |
| 49.9                                           | 6.15                                     |
| 54.9                                           | 6.16                                     |
| 49.0                                           | 1.14                                     |
| 51.2                                           | 2.18                                     |
| 43.0                                           | 3.78                                     |
| Average                                        | 44.09                                    |
|                                                | 3.61                                     |

As aforementioned, the addition of calcium chloride is found to have some beneficial effects for the pyrochlore flotation as clearly illustrated by Example VII following.

## EXAMPLE VII

Two test runs were carried out on the same composite sample similar to that used in Example I. The reagent combination and procedure used were the same as

those used in Example I. One run was carried out without and the other run with calcium chloride addition. The results of the two runs are set forth in Table No. VIII.

Table No. VIII

|                                       | WITHOUT $\text{CaCl}_2$ ADDITION |                           |                                | WITH 10 lbs./ton $\text{CaCl}_2$ ADDITION |                           |                                |
|---------------------------------------|----------------------------------|---------------------------|--------------------------------|-------------------------------------------|---------------------------|--------------------------------|
|                                       | % Wt                             | % $\text{Cb}_2\text{O}_5$ | $\text{Cb}_2\text{O}_5$ Distr. | % Wt                                      | % $\text{Cb}_2\text{O}_5$ | $\text{Cb}_2\text{O}_5$ Distr. |
| Slimes                                | 8.4                              | 0.55                      | 5.2                            | 8.5                                       | 0.48                      | 4.8                            |
| Rejects                               | 72.7                             | 0.074                     | 6.1                            | 80.5                                      | 0.044                     | 4.2                            |
| Pyrite                                |                                  |                           |                                |                                           |                           |                                |
| Concentrate                           | 0.46                             | 0.38                      | 0.2                            | 0.45                                      | 0.25                      | 0.1                            |
| Middlings                             | 17.0                             | 0.32                      | 6.8                            | 9.3                                       | 0.73                      | 8.1                            |
| $\text{Cb}_2\text{O}_5$ Concentration | 1.45                             | 50.2                      | 81.7                           | 1.24                                      | 56.30                     | 82.8                           |
| Feed Calculated                       | 100.0                            | 0.89                      | 100.0                          | 100.0                                     | 0.84                      | 100.0                          |

The cationic collector of the amine type used in combination with the oxalic acid or oxalate salt modifying agent is, as aforementioned, preferably of the diamine acetate type advantageously having a carbon chain length of 10 to 22 carbon atoms. The Duomac-T collector used in the preceding examples has saturated C-16 and C-18 fractions of 29.0 and 23.0% by weight respectively, with smaller amounts of saturated C-12, C-14, C-15 and C-17 fractions totalling 5.5%, and an unsaturated fraction totalling 42.5% by weight. This collector provided the most advantageous results of the diamine acetate collectors used. However, other diamine acetate collectors in the C-10 to C-22 group have proven to be effective also in the process of the

tests. The first series (Direct) was performed following the standard direct flotation procedure used in Example I and the second series (Carbonate Preflotation) 20 was performed using the carbonate prefloat procedure of Example IV. Reagents and procedures used were as in Examples I and IV, respectively. Each Duomac collector was added in a mixture containing 3 parts Duomac and 1 part Ethofat 242/25 in a 1% aqueous solution, as in all the previous examples. Results of the two 25 series of flotation tests are summarized in Table X. Tests 2 and 5 were carried out using a mixture of oxalic and hydrofluoric acids as modifying agent in the ratio of 3 parts oxalic to 1 part hydrofluoric as in Example 30 V.

TABLE X

| TEST<br>No. | FLOTATION<br>PROCESS      | MODIFYING<br>AGENT | COLLECTOR | HEADS<br>% $\text{Cb}_2\text{O}_5$ | CONC.<br>% $\text{Cb}_2\text{O}_5$ | RECOV-<br>ERY<br>% | REAGENT CONSUMPTION LBS/ |      |
|-------------|---------------------------|--------------------|-----------|------------------------------------|------------------------------------|--------------------|--------------------------|------|
|             |                           |                    |           |                                    |                                    |                    | Collector                | Acid |
| 1           | Direct                    | Oxalic             | Duomac T  | 0.94                               | 55.3                               | 66.0               | 1.105                    | 4.75 |
| 2           | Direct                    | Oxalic + HF        | Duomac T  | 0.93                               | 54.8                               | 67.7               | 0.855                    | 4.00 |
| 3           | Direct                    | Oxalic             | Duomac C  | 1.03                               | 55.2                               | 55.3               | 0.97                     | 4.00 |
| 4           | Carbonate<br>Preflotation | Oxalic             | Duomac T  | 0.93                               | 45.5                               | 64.3               | 0.47                     | 3.50 |
| 5           | Carbonate<br>Preflotation | Oxalic + HF        | Duomac T  | 0.90                               | 53.3                               | 70.9               | 0.30                     | 3.25 |
| 6           | Carbonate<br>Preflotation | Oxalic             | Duomac C  | 1.03                               | 57.7                               | 51.7               | 0.47                     | 3.50 |
| 7           | Carbonate<br>Preflotation | Oxalic             | Duomac HH | 0.99                               | 42.1                               | 23.94              | 0.48                     | 3.75 |

Invention and effectiveness of this range of diamine acetate collectors is shown in Example VIII following which gives the results of tests carried out with Duomac-T collector (used in the tests of previous examples) and also Duomac-C (trade mark) and Duomac-HH (trade mark) collectors which have carbon fractions in the C-10 to C-22 range, aforementioned. The carbon chain length distribution of the Duomac-T, Duomac-C and Duomac-HH collectors is set forth in Table No. IX following.

Table IX

| Chain Length Distribution (%) of Collectors<br>Used in Example VIII (Saturated) |          |          |           |
|---------------------------------------------------------------------------------|----------|----------|-----------|
|                                                                                 | Duomac C | Duomac T | Duomac HH |
| C-6                                                                             | 0.5      | —        | —         |
| C-8                                                                             | 8.0      | —        | —         |
| C-10                                                                            | 7.0      | —        | —         |
| C-12                                                                            | 50.0     | 1.0      | —         |
| C-14                                                                            | 18.0     | 3.0      | 6.1       |
| C-15                                                                            | —        | 0.5      | —         |
| C-16                                                                            | 8.0      | 29.0     | 28.1      |
| C-17                                                                            | 1.5      | 1.0      | —         |
| C-18                                                                            | —        | 23.0     | 22.8      |
| C-20                                                                            | —        | —        | 23.0      |
| C-22                                                                            | —        | —        | 19.7      |
| C-24                                                                            | —        | —        | —         |
| Unsaturated<br>Total                                                            | 7.0      | 42.5     | 0         |

45 The Duomac-T collector is seen by the results of Example VIII to be the most effective of those tested. Thus, the diamine acetate group of collector having a carbon chain length of 16 to 18 carbon atoms is most 50 advantageous. However, the Duomac-C collector, with carbon fractions essentially in the C-12 to C-14 range, shows excellent selectivity but with lower recovery in the tests carried out. Less efficiency in terms of selectivity and recovery was found in the Duomac-HH collector having carbon fractions essentially in the C-16 to C-22 range. The tests of Example VIII show, nevertheless, that diamine acetate collectors having different carbon chain length within C-10 to C-22 give reasonable results for pyrochlore flotation, the poorer results obtained with the longer carbon chain collectors being 60 still quite acceptable.

It can be seen that the process of the present invention provides a simple and economical procedure for treating ores containing small amounts of columbium-bearing minerals and large amounts of gangue materials, particularly carbonates, by froth flotation techniques to obtain a high grade  $\text{Cb}_2\text{O}_5$  concentrate.

What we claim is:

1. A process for beneficiating by froth flotation an ore containing small amounts of the columbium-

bearing mineral pyrochlore and large quantities of gangue materials, including large quantities of carbonates from the group comprising dolomite, ankerite, calcite and siderite, which comprises grinding said ore to a small particle size suitable for separation of the columbium-bearing minerals by froth flotation, subjecting an aqueous pulp of the so-ground ore, in the presence of a cationic collector of the diamine acetate type, having a carbon chain length of 10 to 22 carbon atoms, a dispersing agent acting in combination with the collector, a modifying agent providing a source of free oxalate ions from the group consisting of oxalic acid and oxalate salts and at least one depressant from the group consisting of caustic starch and sodium silicate to depress the carbonates in combination with the modifying agent, to froth flotation at a pH of below 7 and forming a concentrate rich in the columbium-bearing minerals and a columbium-lean tailing and collecting said concentrate.

2. A process as claimed in claim 1 wherein the diamine acetate collector has a carbon chain length of in the order of 16 to 18 carbon atoms.

3. A process as claimed in claim 1, wherein calcium chloride is included as a modifying agent in the flotation treatment in promoting the pyrochlore.

4. A process as claimed in claim 1, wherein the gangue materials include heavy minerals from the group comprising ilmenite, hematite and magnetite and at least one depressant from the group consisting of caustic starch and lactic acid is used to depress the heavy minerals.

20  
25  
30

5. A process for beneficiating by froth flotation an ore containing small amounts of the columbium-bearing mineral pyrochlore and large quantities of gangue materials, including large quantities of carbonates, which comprises grinding said ore to a small particle size suitable for separation of the columbium-bearing minerals by froth flotation, subjecting an aqueous pulp of the so-ground ore, in the presence of a cationic collector of the diamine acetate type, having a carbon chain length of 10 to 22 carbon atoms, a dispersing agent acting in combination with the collector, a modifying agent providing a source of free oxalate ions from the group consisting of oxalic acid and oxalate salts, at least one gangue depressant from the group consisting of caustic starch, sodium silicate and lactic acid to depress the carbonates in combination with the modifying agent, and an inorganic acid from the group consisting of HF,  $H_2SO_4$ , HCl and  $H_3PO_4$ , to froth flotation at a pH of below 7 and forming a concentrate rich in the pyrochlore mineral and a columbium-lean tailing and collecting said concentrate.

6. A process as claimed in claim 5, wherein oxalic acid is used as the modifying agent.

7. A process as claimed in claim 5, wherein hydrofluoric acid is included as a modifying agent in the flotation treatment.

8. A process as claimed in claim 5, wherein calcium chloride is included as a modifying agent in the flotation treatment in promoting the pyrochlore.

\* \* \* \* \*

35

40

45

50

55

60

65